

1

3,455,713

FLAME-RETARDANT REGENERATED  
CELLULOSE

Leonard E. A. Godfrey, Franklin Township, Somerset County, N.J., assignor to FMC Corporation, Philadelphia, Pa., a corporation of Delaware  
No Drawing. Filed July 21, 1966, Ser. No. 566,757  
Int. Cl. D01f 3/12; C09j 3/04; C08b 21/20  
U.S. Cl. 106—165 10 Claims

## ABSTRACT OF THE DISCLOSURE

Permanently flame-retardant regenerated cellulose filaments and filamentary articles containing dispersed therein a flame-retardant amount of a substantially water-insoluble, liquid phosphonitrilate polymer, and a method of preparing the filamentary articles are disclosed herein.

It is desirable, for many textile purposes to provide cellulose fibers and yarns having greatly decreased flammability. The production of rayon which demonstrates permanent and acceptable flame-retardant properties for all textile requirements, using inexpensive and commercially suitable chemical flame-retardants, has not been accomplished to date.

The application of various organic and inorganic flame-retardants to the surface of cellulose fibers and fabrics has not produced the desired result for a number of reasons. In many instances, the chemical flame-retardant is effectively removed when the fabric is washed with water or dry cleaned with solvents. Other flame-retardant chemicals which may be applied to the fabric surface and retained after washing are generally too costly. In other cases, the chemicals used may provide some lasting reduction in flammability but destroy fiber and fabric characteristics, such as tenacity, softness, whiteness, and dyeability, which are desirable and necessary for textile applications.

In the manufacture of rayon by the viscose method, it has been proposed to add various flame-retardant chemicals to the viscose prior to spinning. This approach presents many additional problems because of the particular chemistry of the viscose process. Accordingly, the flame-retardant must be stable and inert with respect to the highly alkaline viscose and also with respect to the acid regenerated bath into which the viscose is extruded. It must not be extracted during spinning and processing. Furthermore, the added material must not interfere with the spinning process, i.e., cause clogging of the spinnerets. The rayon produced from the flame-retardant containing viscose must not be degraded in any of its properties and must have a substantial and permanently reduced flammability after continued washing and cleaning.

It is an object of this invention to provide a permanently flame-retardant rayon fiber without appreciable degradation of any fiber properties.

It is another object of this invention to provide a flame-retardant rayon textile that will retain its flame-retardant property after continued washing with alkaline soap and detergents in water or after dry cleaning with organic solvents.

It is still another object of this invention to provide a flame-retardant rayon that is not adversely affected by exposure to ultra-violet light or bleaching solutions.

It is a further object of this invention to provide a process for preparing a permanently flame-retardant rayon fiber.

These and other objects are achieved in accordance with this invention which comprises a regenerated cellulose filament having dispersed therein a substantially

2

water-insoluble, liquid phosphonitrilate polymer having the following general formula:



wherein R and R' are the same or different alkyl or alkenyl radicals having from one to six carbon atoms and n in an integer of at least three. For example, R and R' include methyl, ethyl, propyl, isopropyl, butyl, isobutyl, amyl, isoamyl, hexyl, allyl, and crotyl radicals. In a preferred embodiment of this invention R and R' are n-propyl, isopropyl or allyl radicals since polymers wherein both R and R' have fewer carbon atoms tend to be more water-soluble, whereas the presence of more carbon atoms provide products having a lower phosphorous content thereby reducing their effectiveness as flame retardants. This can be overcome, of course, by using polymers wherein R contains fewer carbons and R' contains more. For example, R is methyl or ethyl and R' is butyl, amyl, isoamyl, or hexyl.

The liquid phosphonitrilate polymer is a cyclic trimer, tetramer or higher cyclic polymer, or a linear polymer and is preferably employed as a mixture of these isomers for economic reasons. It has been found, however, that the pure polymeric isomer is just as effective as the mixture for the purposes of this invention.

The amount of phosphonitrilate flame-retardant dispersed in the regenerated cellulose filament varies from about 1 to about 30% and preferably from 2 to 20%, based on the weight of the filament.

The method of this invention comprises incorporating the above described liquid phosphonitrilate in a viscose solution and spinning the viscose in the shape of one or more filaments into a coagulating and regenerating medium. The formed filaments are aftertreated using techniques well-known in the rayon field to provide continuous filaments, fibers and yarn, as well as staple fibers. These may then be used to prepare any known textile article in which the flame-retardant property is desirable.

The flame-retardant phosphonitrilate of this invention is a liquid of pumpable consistency which is preferably used as a crude reaction product, prepared, for example, in a known manner by the conversion of the corresponding polymeric phosphonitrilic chlorides to the specified esters; or in a distilled or otherwise refined state. If desired, suitable solutions of the phosphonitrilate may also be prepared and used for incorporation in viscose.

In a preferred embodiment of the method of this invention, a controlled amount of the flame-retardant phosphonitrilate is injected into the viscose just prior to its extrusion through the spinnerets. The viscose is extruded into an acid bath and processed in a conventional manner.

The following example is set forth to demonstrate the method and product of this invention.

## EXAMPLE

Excellent flame-retardant rayon yarn with no after-glow was produced from viscose comprising 8.2% cellulose, 6.2% sodium hydroxide and 34.0% carbon disulfide, based on the weight of the cellulose, having a common salt test range of 3.5 to 7.3 and a Ball-Fall range of 52 to 100 seconds at 18° C.

A metered amount, based on the weight of the cellulose in the viscose of a liquid mixture of di-n-propyl phosphonitrilate polymers, as defined for this invention, comprising about 65% trimer, about 15% tetramer, between about 15 and 20% of higher cyclic polymers and less than about 5% of linear polymers, was pumped into the viscose line supplying the spinnerets.

The flame-retardant containing viscose was spun into

a bath comprising 9.0% sulfuric acid, 2.0% zinc sulfate and 15.0% sodium sulfate at 55° C. and then further processed by a series of baths including water wash, desulfurization, bleaching, bleach acid, anti-chlorine, and soft finish. The yarn was dried and collected.

A yarn flammability test was conducted with yarn produced as described above. The test consisted of first preparing a yarn bundle by wrapping the yarn around the closed fingers of an extended hand to produce a bundle of 6000 denier and then removing it from the hand. The yarn bundle is twisted five times and then doubled on itself to produce an integrated yarn bundle, one and one-half inches long and of 12,000 denier size. The free ends of the yarn bundle are clamped in forceps, and the bundle, held in horizontal position, is passed through the tip of the flame of a Fisher burner in an oscillating motion at a rate of one pass per second. The burner flame is adjusted to a two inch height and a blue flame. The number of passes to induce flaming of the sample is determined. A control yarn bundle (yarn contains no flame-retardant) inflames in 1 or 2 passes and flame-retardant yarns are classified for inflammability as follows:

|                   |                         |
|-------------------|-------------------------|
| 1-2 passes        | Poor.                   |
| 3-4 passes        | Fair.                   |
| 5-6 passes        | Good.                   |
| 7-8 passes        | Very good to excellent. |
| 10 or more passes | Excellent.              |

Rayon yarns, prepared as described above, containing 20, 15, and 12% of the flame-retardant, based on the weight of the cellulose, all were rated excellent in the above test procedure with no evidence of after-glow. After-glow represents combustion without a visible flame.

The filaments of this invention, in the form of yarns, were tested for strength characteristics before and after complete processing. Complete processing involves treating the wet spun yarn in a series of baths as follows: Water wash, desulfurization, water wash, bleaching, water wash, bleach acid, water wash, antichlorine, water wash, and soft finish. Yarns tested before complete processing were merely subjected to one water wash after spinning.

The following table sets forth the data obtained from these strength tests with yarns prepared as described in the foregoing example.

TABLE I

| Percent phosphonitrilate | Processing | Denier/filament | Yarn denier | Tc   | Ec   | Tw   | Ew   |
|--------------------------|------------|-----------------|-------------|------|------|------|------|
| 0.0                      | Complete   | 300/60          | 291         | 2.5  | 18.6 |      |      |
| 12.0                     | Water-wash | 300/60          | 318         | 2.07 | 20.1 | 1.09 | 24.2 |
| 12.0                     | Complete   | 300/60          | 324         | 1.89 | 20.2 | 1.01 | 24.2 |
| 15.0                     | Water-wash | 300/60          | 331         | 1.80 | 18.7 | 0.96 | 22.2 |
| 15.0                     | Complete   | 300/60          | 402         | 1.59 | 18.8 | 0.82 | 22.7 |
| 20.0                     | Water-wash | 300/60          | 336         | 1.76 | 18.9 | 0.91 | 23.0 |
| 20.0                     | Complete   | 300/60          | 331         | 1.88 | 19.6 | 0.98 | 23.5 |

Tc=Conditioned tenacity; Ec=Conditioned elongation; Tw=Wet tenacity; Ew=Wet elongation.

Yarn physical characteristics, as compared to similar yarn containing no flame-retardant are excellent even after complete processing.

These yarns were also studied to determine the effect of ultra-violet light thereon. The tests were conducted with a Fadeometer under the same conditions for each yarn sample. The data developed are given in the following table.

TABLE II

| Percent phosphonitrilate | Percent loss in yarn strength |           |
|--------------------------|-------------------------------|-----------|
|                          | 50 hours                      | 100 hours |
| 0.0                      |                               | 12.0      |
| 12.0                     | 7.6                           | 9.2       |
| 15.0                     | 3.3                           | 6.6       |
| 20.0                     | 4.6                           | 9.3       |

The ultra-violet light strength stability of the flame-retardant yarns is even better than the control sample, further demonstrating unexpected results for this invention.

75

Retention of the flame-retardant in the yarn and fabrics produced therefrom is of primary importance and this property of the yarns of this invention was given severe testing. Yarn, and fabric produced therefrom, containing 12.0% of the liquid phosphonitrilate polymer of this invention as disclosed in the foregoing example, based on the weight of the cellulose, were examined for the retention of the flame-retardant.

The following table sets forth the retention data obtained.

TABLE III

| Processing:                         | Percent retention <sup>1</sup> |
|-------------------------------------|--------------------------------|
| Complete (as described for Table I) | 93.8                           |
| Soxhlet Extractions:                | Percent loss <sup>2</sup>      |
| 10 cycles—water                     | 3.2                            |
| 20 cycles—petroleum ether           | 2.9                            |
| 20 cycles—perchloroethylene         | 7.2                            |
| Commercial laundering: <sup>3</sup> | Percent loss <sup>2</sup>      |
| 20 cycles                           | 12.0                           |

<sup>1</sup> Retention of amount of flame-retardant injected in viscose based on phosphorous analysis.

<sup>2</sup> Loss from completely processed yarn based on phosphorous analysis.

<sup>3</sup> Fabric prepared from completely processed yarn washed in automatic washer with  $\frac{1}{4}$  cup of sodium oleate per cycle.

Yarns and fabrics subjected to the above test procedures all retain their excellent flame-retardant properties.

A summary of some of the advantages of this invention includes the following points.

The flame-retardant of this invention is a fairly mobile liquid that can be readily pumped and metered into a viscose solution. Thus, there is no need to make alkaline solutions or dispersions which may cause spinning problems.

The initial retention of the flame-retardant on spinning into cellulose filaments and fibers is excellent in contrast to many hydrolyzable or water-soluble fire-retardants. Surprisingly, there is little or no hydrolysis of this flame-retardant even when mixed with viscose and allowed to stand for up to 18 hours.

There is almost no loss in the alkaline desulfurization and anti-chlorine baths that are conventionally used in processing rayon. Alkali-soluble materials tend to be leached from the rayon during processing.

The retention is excellent after many launderings and dry cleanings.

The fire-retardancy of the product of this invention is excellent despite the absence of halogens which often cause ultra-violet light degradation.

Unlike many other nitrogen containing compounds, the liquid phosphonitrilate polymer of this invention has no tendency to pick up chlorine from bleaching solutions which might lead to yellowing and fiber degradation.

The phosphonitrilate polymer is dispersed readily and evenly throughout the fiber because of its liquid nature, and therefore, has little effect on the fiber tensile strength. Such small losses in strength that do occur generally result only from displacement of a certain amount of cellulose.

The appearance and general physical properties of the flame-retardant rayon of this invention differ only slightly from ordinary rayon. Hence, the fibers can be processed in the normal fashion.

Various changes and modifications may be made prac-

ticing the invention without departing from the spirit and scope thereof and, therefore, the invention is not to be limited except as defined in the appended claims.

I claim:

1. Regenerated cellulose filaments and filamentary articles, said filaments having dispersed therein a flame-retardant amount of a substantially water-insoluble, liquid phosphonitrilate polymer having the following general formula:



wherein R and R' are alkyl or alkenyl radicals having from 1 to 6 carbon atoms and n is an integer of at least 3. 15

2. The regenerated cellulose filaments of claim 1 containing from about 1 to about 30%, based on the weight of the cellulose, of the liquid phosphonitrilate polymer.

3. The regenerated cellulose filaments of claim 1 wherein R and R' are the same and contain 3 carbon atoms. 20

4. The regenerated cellulose filaments of claim 3 wherein R and R' are n-propyl radicals.

5. The regenerated cellulose filaments of claim 3 wherein R and R' are isopropyl radicals.

6. The regenerated cellulose filaments of claim 3 wherein R and R' are allyl radicals.

7. A method of preparing a permanently flame-retardant regenerated cellulose filament which comprises mixing viscose and a flame-retardant amount of a substantially water-insoluble, liquid phosphonitrilate polymer having the following general formula:



wherein R and R' are alkyl or alkenyl radicals having from 1 to 6 carbon atoms and n is an integer of at least 3, shaping the mixture into a filament, and coagulating and regenerating said filament.

5 8. The method of claim 7 wherein the viscose is passed under pressure to a spinneret and extruded, and the liquid phosphonitrilate polymer is injected at a controlled rate into the viscose prior to extrusion.

9. The method of claim 7 wherein from about 1 to about 30% of the liquid phosphonitrilate is mixed with the viscose, based on the weight of the cellulose in the viscose.

10 10. The method of claim 7 wherein R and R' are the same and contain 3 carbon atoms.

#### References Cited

##### UNITED STATES PATENTS

|           |        |                 |       |           |
|-----------|--------|-----------------|-------|-----------|
| 2,192,921 | 3/1940 | Lipkin          | ----- | 260—927   |
| 3,266,918 | 8/1966 | Schappel et al. | ----- | 106—15 XR |
| 3,370,020 | 2/1968 | Allcock et al.  | ----- | 260—2     |

JULIUS FROME, Primary Examiner

L. HAYES, Assistant Examiner

##### U.S. CL. X.R.

106—15, 168, 177; 252—8.1; 264—194

UNITED STATES PATENT OFFICE  
CERTIFICATE OF CORRECTION

Patent No. 3,455,713

July 15, 1969

Leonard E. A. Godfrey

It is certified that error appears in the above identified patent and that said Letters Patent are hereby corrected as shown below:

Column 3, line 27, "7-8" should read -- 7-9 --.

Signed and sealed this 18th day of November 1969.

(SEAL)

Attest:

Edward M. Fletcher, Jr.

Attesting Officer

WILLIAM E. SCHUYLER, JR.

Commissioner of Patents